

Nov. 24, 1953

W. T. KNOX, JR

2,660,553

## WAX COMPOSITION AND PROCESS FOR PRODUCING WAX

Filed Feb. 23, 1951



William T. Knox Jr. Inventor

By W. O. T. Heilman attorney

## UNITED STATES PATENT OFFICE

2,660,553

WAX COMPOSITION AND PROCESS FOR  
PRODUCING WAX

William T. Knox, Jr., Cranford, N. J., assignor  
to Standard Oil Development Company, a cor-  
poration of Delaware

Application February 23, 1951, Serial No. 212,295

5 Claims. (Cl. 196—17)

1

This invention concerns wax having novel and unusual physical properties derived from a novel combination of processing steps. In accordance with this invention, a uniquely desirable wax is obtained by subjecting the "cycle oil" obtained from catalytic cracking operations to a solvent extraction operation after which the raffinate of the extraction operation is de-waxed to provide the final wax product. The wax thus obtained is characterized by a hardness and flexibility peculiarly adapting the wax for application in food wrapping services and for other uses.

While wax may be obtained in a number of ways following differing processing techniques, at the present time most waxes are obtained by de-waxing distillate fractions of crude oil such as the lubricating oil fraction. It is now generally appreciated that the conventional paraffin wax obtained from this source is characterized by the presence of hydrocarbons which are predominantly normal paraffins. Wax obtained by the de-waxing of lubricating oil stocks, presumably by virtue of its hydrocarbon composition, is for many purposes unduly inflexible. High flexibility has been found to be related to good performance of waxes as coating material at low temperatures. Hardness is again an important characteristic governing in part the ability of the wax to withstand rough handling and chipping. Flexibility and hardness control the permeability characteristics of a wax coating, since the two properties in combination materially aid in preventing breakage of the wax film and the consequent moisture leakage which can occur on breakage. As a result of these factors, for many applications and in particular for the coating of paper used in packaging food, it is desirable to secure wax having high flexibility while being comparatively hard in nature. It is therefore the principal object of this invention to provide a novel type of wax having improved properties of hardness and flexibility.

As herein disclosed, a flexible wax having desirable hardness may be obtained by a processing sequence applied to the gas oil fraction of a crude petroleum oil. The gas oil fraction of crude petroleum, boiling in the range of about 700 to 1100° F. is first subjected to a catalytic cracking operation. The heaviest boiling oil obtained from the catalytic cracking, that is, boiling in the range of about 700 to 1100° F., is then subjected to a treating operation to selectively remove the more aromatic constituents. This may be accomplished by a selective absorption process utilizing an absorbent such as silica gel, acti-

vated coke, clay, etc. Alternatively, the aromatic constituents may be selectively removed by a solvent extraction operation employing a solvent which selectively removes the aromatics, leaving a raffinate substantially free of aromatics. This intermediate product, substantially free of aromatics, is then subjected to a de-waxing operation so as to permit the recovery of wax therefrom. It is this wax which has the unusual properties referred to.

On analysis and by way of a theoretical explanation of what is involved, it appears that the wax obtained from this processing sequence is characterized by hydrocarbon constituents which are more cyclic or isoparaffinic in nature than in the case of ordinary conventionally refined wax. The processing sequence followed is of a nature to provide this result. It is significant that waxes obtained by this processing technique are materially different than the naturally occurring paraffin waxes or micro-crystalline waxes. In effect the processing employed to provide the waxes of this invention is effective to synthesize a wax differing from normal wax characteristics as a result of the cracking and aromatic extraction procedures employed.

To fully disclose the nature of this invention and the manner in which the invention is practiced, reference is made to the accompanying drawing, illustrating a diagrammatic flow plan of the process to be followed in obtaining the novel wax of this invention.

Referring now to the drawing illustrating the entire integral process to be employed, numeral 1 designates a crude petroleum distillation zone. A crude petroleum oil such as a mixed base crude oil is introduced to distillation zone 1 through line 2. The distillation operation is conducted to permit removal of volatile fractions overhead through line 3 and of heavier boiling products such as gasoline, kerosene and heating oils through side stream withdrawals 4, 5, 6, and so on. The heavier boiling fractions having initial boiling ranges of from 800 to 1100° F. and higher are withdrawn as a side stream product through line 7. It is particularly contemplated that in the practice of this invention, distillation zone 1 be of such a nature as to provide a higher boiling fraction boiling in the range of about 700 to 1100° F., preferably as obtained by vacuum distillation operations. This fraction is then conducted to a catalytic cracking zone identified by the rectangle 8. The cracking operation to be conducted in zone 8 is of any desired type

employing a catalyst such as modified natural or synthetic clay or gel type catalysts. Examples of these are montmorillonite clays, silica-alumina, silica-magnesia composites, and other conventional cracking catalysts. The operation may be of a continuous or batch nature employing fixed beds, moving beds, fluidized, or suspensoid systems. The heat required for cracking may be supplied as preheat of processed materials and/or as the sensible heat of exothermically regenerated catalyst or in any other conventional manner. The cracking is carried out at temperatures of about 800 to 1000° F., and pressures of about atmospheric to 25 p. s. i. g., or higher. The total cracked products are removed from cracking zone 8 and are conducted to a product fractionator 9. Fractionator 9 is operated to remove lighter fractions of the cracked products through overhead 10, side streams 11, 12 and so on. A bottoms product is obtained from fractionator 9 which may be removed through line 14. In the event the cracking operation conducted in zone 8 was of a fluidized nature, the material withdrawn through line 14 will contain a small percentage of catalyst particles carried over from zone 8. In this case, it is necessary to pass the product stream of line 14 to a settler 15 or otherwise to process the stream to permit separation of the liquid hydrocarbon product from the catalyst. Thus, a clarified hydrocarbon stream is removed from zone 15 through line 16. For the purposes of this invention, the bottoms product of fractionator 9, corresponding to the stream of line 14 or 16, boils in the range of about 700 to 1100° F. The stream of line 16 is generally called cycle oil. As the name suggests, cycle oil is generally recycled to the cracking zone, as heretofore virtually no other use has been found for this oil. However, it should be appreciated that return of cycle oil to the cracking operation is not particularly desirable. Cycle oil is refractory in nature and constitutes a very poor cracking feed, causing substantial deposition of carbon and coke on the catalyst employed during cracking. As will be appreciated therefore, it is one of the features of this invention to employ cycle oil so as to prevent recycling to a cracking operation and so as to provide valuable products.

As the conduct of the process as described heretofore is well known to the art, no further description of this phase of the process is considered necessary. The cycle oil of line 16, derived as indicated, is then conducted to a zone for the selective removal of aromatic constituents. As formerly suggested, this zone may employ an adsorbent such as silica gel which will selectively adsorb aromatic constituents. The aromatic constituents may be removed by adsorbent treatment in fixed bed or counterflow operations as well known to the art. Alternatively, the aromatic constituents may be selectively removed by a solvent extraction operation. It is this specific embodiment of the invention which is illustrated in the drawing. Thus, in order to remove the aromatic constituents by solvent extraction, the stream of line 16 is conducted to solvent extraction zone 19. Zone 19 may be arranged as a countercurrent liquid-liquid contacting tower, if desired, provided with pierced plates, packing, or other means for securing efficient liquid-liquid contacting of the oil and the solvent employed.

As is well known, a variety of solvents may be employed to secure the desired selective removal

of aromatic constituents. Thus, for example, sulfur dioxide, phenol, furfural, nitrobenzene, ammonia and other solvents, alone or in conjunction with solvent modifiers, may be employed. While the contacting of the solvent and oil may be conducted in any desired contacting equipment of a batch or continuous nature, countercurrent treating technique is preferably employed. In such a system, the oil feed of line 16 is introduced to a countercurrent contacting tower 19 at a point near the bottom thereof. A solvent such as phenol is introduced at an upper portion of the tower through line 20. About a 150 to 350 volume percent treat is used. The oil passes upwardly through the tower while the solvent passes downwardly through the tower, permitting removal from the bottom of the tower of what is known as an extract phase through line 21. The extract phase will consist principally of the solvent such as phenol together with the constituents selectively extracted from the oil consisting principally of aromatic hydrocarbons. The extract phase may be disposed of as desired. In fact, the hydrocarbons contained in the extract phase are valuable in providing a source of aromatic hydrocarbons suitable for use as plasticizers, fluxing agents, etc. The material withdrawn from the top of tower 19 through line 22 is known as the raffinate phase and consists principally of the initial oil feed minus the aromatic constituents originally present in the feed, admixed with small proportions of the solvent employed during the contacting. The raffinate phase withdrawn from solvent extraction zone 19 through line 22 is then passed to dewaxing zone 30. The de-waxing operation conducted in zone 30 may be chosen from any of the conventional de-waxing processes of a nature to reduce the wax content of the hydrocarbon fraction treated to any desired extent. In general, it is preferred that a solvent de-waxing operation be employed. For example, the hydrocarbon oil of line 22 may be diluted with about 2 to 4 parts per volume with a solvent such as propane or methyl ethyl ketone, including a minor portion of aromatic hydrocarbons such as benzene or toluene if desired. Any aliphatic ketone, or mixtures thereof, having from three to six carbon atoms may be employed as the de-waxing solvent. The mixture of hydrocarbon oil and solvent is then heated sufficiently to secure the solution of all wax present. A temperature of about 150° F. is generally suitable. Thereafter, the mixture of oil and solvent is cooled to a temperature of about 25° F. to -40° F., so as to secure the crystallization of the wax present. The chilled mixture of oil, solvent and wax is then filtered to eliminate this wax, permitting removal from zone 30 of a dewaxed hydrocarbon oil, and permitting removal from zone 30 of a wax product. It may be observed that the dewaxed hydrocarbon oil is a valuable lubricating oil stock characterized by a high viscosity index. Alternatively, if desired, this dewaxed raffinate may be employed as a cracking stock, being well adapted for cracking and being free of the disadvantages characteristic of cycle oil. The wax obtained from the dewaxing zone 30 is suitable for use as the final product of this process. The wax is then subjected to further refining operations such as solvent de-oiling, to reduce the oil content of the wax, percolation for color and odor improvement, or other conventional finishing processes.

As a specific example of this invention, a gas

oil was subjected to a fluidized catalytic cracking operation. The gas oil boiled in the range of about 650° to 1100° F., and was derived from a mixture of West Texas and similar types of crude oil. The products of the catalytic cracking operation were fractionated and treated to provide a clarified oil boiling in the range of 700° to 1100° F. This clarified oil was then subjected to contact with a selective solvent consisting of phenol containing 7% of water as a solvent modifier. Contact was carried out in a contacting tower providing seven extraction stages while injecting 2.8% of water at the raffinate outlet end of the extraction system; a 160% treat of solvent by volume based on the feed was employed. The raffinate from this extraction operation was topped so as to secure the fraction boiling in the range of 700° to 1100° F.; thereafter the raffinate was dewaxed by mixing the raffinate with 300 volume percent of secondary butyl acetate, heating to about 120° F., and cooling to 0° F. The wax thus precipitated was filtered and remixed with 3 volumes of secondary butyl acetate at 0° F., thereafter the wax was filtered from this mixture as the final product.

Data relative to this experiment are given in Table I below, showing the yield and inspections of the different products obtained.

TABLE I  
*Extraction and dewaxing of catalytic cycle stock*

|                                | Feed  | Extract | Raffinate |        |                |       |
|--------------------------------|-------|---------|-----------|--------|----------------|-------|
|                                |       |         | Waxy      | Topped | Dewaxed topped | Wax   |
| Yield on feed, volume percent. | 100   | 67.3    | 32.7      | 31     | 22             | 9     |
| Inspections:                   |       |         |           |        |                |       |
| Gravity, °API                  | 9.7   | -0.2    | 35.3      | 34.7   | 32.1           | ----- |
| Flash, °F., COC                | 340   | 380     | 370       | 415    | 430            | ----- |
| Viscosity at 100° F., SSU      | 1,208 | 1,340   | 1,106     | 1,117  | 162            | ----- |
| Viscosity at 210° F., SSU      | 43.6  | 59.8    | 41.1      | 42.2   | 44.4           | 38.5  |
| Viscosity index                | +24   | -----   | -----     | -----  | 106            | ----- |
| Pour, °F                       | +95   | +80     | +110      | +110   | +15            | ----- |

<sup>1</sup> Extrapolated values.

For comparative purposes the corresponding inspections of a conventional refined wax derived from dewaxing of the lubricating oil cut of a crude petroleum oil and of a microcrystalline wax are also given.

by holding one end firmly in a vise in a vertical position and displacing the strip with a micrometer at a distance of one inch from the vise jaws until the first sign of a crack appears in the strip.

The micrometer extension required is recorded and the thickness of each specimen is measured. Six samples are broken for each thickness determined; three of the samples are broken with the air cooled side facing the micrometer, and three samples are broken with the water cooled side facing the micrometer. The micrometer extension determined in this test is expressed in thousandths of an inch and is reported as flexibility.

The hardness test was conducted employing an Abraham consistometer of the nature described in the "Chemistry and Technology of Waxes," published by the Reinhold Publishing Company.

In considering the data shown in Table II, it may be noted that the catalytic wax obtained in accordance with this invention is similar to paraffin waxes in melting point and refractive index, but differs somewhat in viscosity and specific gravity. Most important, however, the wax of this invention is greatly different from paraffin wax in flexibility although having comparable hardness. The fact that the two wax compositions are actually materially different is also borne out by the higher mid-boiling point of the

wax of this invention as compared to conventional refined paraffin wax.

In comparing the wax of this invention to micro-crystalline wax, it may be noted that the waxes are similar in melting point, oil content

TABLE II

|                                      | Catalytic | Refined     | Microcrystalline |
|--------------------------------------|-----------|-------------|------------------|
| Melting point, °F. (ASTM)            | 134       | 134-135     | 136              |
| Percent oil, ASTM                    | 1.7       | 0.3-0.4     | 2.4              |
| Refractive index at 153° F. (67° C.) | 1.433     | 1.434-1.435 | 1.442            |
| Specific gravity (60° F., liquid)    | 0.818     | 0.809       | 0.842            |
| Flexibility at 73° F., 0.001"        | 450       | 66-70       | >750             |
| Abraham hardness at 100° F.          | 19.4      | 15-25       | <10              |
| Viscosity at 210° F. (cs.)           | 3.7       | 3.8         | 6.6              |
| Distillation at 1 min., °F.:         |           |             | 13.1             |
| 5% at                                | 422       | 380         | 460              |
| 50% at                               | 460       | 425         | 510              |
| 95% at                               | 620       | 490         | 620              |
| 5 to 95%, °F.                        | 198       | 110         | 160              |
|                                      |           |             | 175              |

The properties of particular interest reported in Table II are the flexibility and hardness of the waxes. The flexibility test employed was conducted by forming a wax disc by pouring a weighed sample of wax on the surface of boiling distilled water in a crystallizing dish providing a given surface area. The wax is then allowed to cool for two to three hours and the discs are then cut into strips 3" x 5". The strips are then placed on a smooth brass plate and cooled to 40° F. in a cold room for 16 hours. A wax strip is broken

65 and boiling range. However, the waxes differ greatly in refractive index, specific gravity, and viscosity. The waxes of this invention are also not nearly as soft and tacky as micro-crystalline waxes.

70 As described therefore, the process of this invention concerns the steps of catalytically cracking a gas oil feed stock; selectively removing aromatic constituents from the cycle oil obtained from catalytic cracking; and thereafter segregating wax from the intermediate product remain-

ing after removal of the aromatic constituents. As emphasized, the wax obtained is unusual as regards its properties of hardness and flexibility, differing materially in these characteristics from waxes obtained by conventional processing.

What is claimed is:

1. A process for producing a moderately hard flexible wax comprising the steps of catalytically cracking a gas oil feed stock boiling in the range of about 650-1100° F., fractionating an oil fraction from the cracked products boiling in the range of about 700-1100° F., selectively removing aromatic compounds from the said oil fraction, and thereafter segregating wax from the said fraction remaining after selective removal of aromatic compounds including the step of de-oiling the said wax.
2. The process defined by claim 1 in which the said selective aromatic removal is conducted by solvent extraction.
3. The process defined by claim 1 in which the said selective aromatic removal is conducted by adsorbent treating.

4. In the production of wax, the improvement which comprises segregating wax from catalytic cracking cycle stock boiling in the range of about 700° to 1100° F. which has been treated to selectively remove aromatic constituents and de-oiling the said segregated wax.

5. A wax having a melting point of about 134° F., a refractive index at 153° F. of about 1.43, a specific gravity (liquid at 60° F.) of about 0.82, an Abraham hardness at 100° F. of about 20, a flexibility at 73° F. of about 450, and a mid-boiling point at 1 mm. mercury of about 460° F.

WILLIAM T. KNOX, JR.

References Cited in the file of this patent

UNITED STATES PATENTS

| Number    | Name             | Date          |
|-----------|------------------|---------------|
| 1,937,518 | Henderson et al. | Dec. 5, 1933  |
| 2,017,432 | Bahlike          | Oct. 15, 1935 |
| 2,127,668 | Adams et al.     | Aug. 23, 1938 |
| 2,378,762 | Frey             | June 19, 1945 |
| 2,429,875 | Good et al.      | Oct. 28, 1947 |